

## UNITED STATES PATENT OFFICE

2,436,272

## MINERAL OIL COMPOSITION

George H. S. Snyder, Woodbury, Ralph V. White, Pitman, John H. Bishop, Wenonah, and John F. Socolofsky, Woodbury, N. J., assignors to Socony-Vacuum Oil Company, Incorporated, a corporation of New York

No Drawing. Application February 27, 1945,  
Serial No. 580,074

10 Claims. (CL 252—56)

1

This invention has to do with lubricants and, more particularly, has to do with lubricants for ferrous metal surfaces in an environment where such surfaces are also subject to contact with water and in consequence are likely to rust.

As is well known to those familiar with the art, difficulties have been experienced during the operation of steam turbines and particularly during the initial operation of new steam turbines because of the rusting of the ferrous metal parts. The combination of fresh (not previously used) oil, clean new metal surfaces, and moist conditions of operation of new steam turbines appears to be particularly conducive to rusting difficulties. Particles of rust deposited on or carried to bearing surfaces of small clearance such as the governor, for example, tend to cause sticking which renders them inoperative. In cases of severe rusting bearings may be injured.

The aforesaid rusting phenomenon is evidently the result of improper or inadequate "wetting" of the metal surfaces with oil thus permitting a preferential contact of the surfaces with the water which is present. Numerous materials have been proposed for use in such oils to counteract the inadequate "wetting" effect; unfortunately, however, such materials have generally given rise to other undesirable phenomena. For example, many organic esters which have been suggested for use in turbine oils and the like to correct the rusting action normally characteristic thereof, have proven to be undesirable inasmuch as they form emulsions with the oil and water present in the environment in which they are used. As is well known, emulsions seriously reduce or impair the high degree of lubricating efficiency required in turbine operation and are to be religiously avoided. Typical of the organic esters which inhibit the rusting action of turbine oils and the like but which give rise to emulsions are those obtained by reaction of alcohols and oxy-polycarboxylic acids; representative of such esters is dioleyl malate.

The present invention is directed to an outstanding mineral oil which is substantially free from the aforesaid rusting and emulsion difficulties. The outstanding mineral oil of this invention comprises a viscous mineral oil having in admixture therewith a small amount of an ester of malic acid obtained by reacting one molar equivalent of malic acid with from about 0.8 to about 1.6 molar equivalents of a short-chain alcohol having from six to eight carbon atoms and with from about 1.2 to about 0.4 molar equivalent of a long-chain alcohol having at least twelve carbon atoms. The present invention is also predicated upon the discovery of an oil similarly characterized comprising a viscous mineral oil containing a small amount of a mixture of esters of malic acid, one of said esters having two short-chain aliphatic groups containing

2

from six to eight carbon atoms substituted for the carboxylic hydrogen atoms of malic acid and being present in the mixture in a molar quantity of from about 40% to about 80%, and another of said esters having two long-chain aliphatic groups containing at least twelve atoms substituted for the carboxylic hydrogen atoms of malic acid and being present in the mixture in a molar quantity of from about 60% to about 20%. Particularly preferred herein, however, are those oils which contain a malic ester having equimolecular proportions of a short-chain aliphatic group and of a long-chain aliphatic group of the type defined above; and those oils which contain a mixture of malic esters in which one of the said esters has two short-chain aliphatic groups and another of said esters has two long-chain aliphatic groups of the type defined above, the esters being present in the mixture in equimolecular proportions. It will be apparent, therefore, that chemical and physical mixtures of such esters, characterized as described above, are contemplated by the present invention.

The short-chain aliphatic groups which contain from six to eight carbon atoms may be wholly saturated or partially saturated and may be either straight- or branched-chain or cyclic in structure, although a wholly saturated branched-chain group such as 2-ethyl hexyl is preferred. Specific examples of such groups are n-hexyl, cyclohexyl, n-heptyl, n-octyl and the preferred 2-ethyl hexyl group. Correspondingly, long-chain aliphatic groups which contain at least twelve carbon atoms, and preferably from twelve to eighteen carbon atoms, may be wholly saturated or partially saturated and may be either straight- or branched-chain in structure and, of such groups the normal, partially saturated group oleyl is preferred. Illustrative of such groups are lauryl, 7-ethyl-2-methyl undecyl, cetyl, oleyl and stearyl. It will be apparent to those familiar with the art that the foregoing aliphatic groups may be introduced into the malic esters contemplated herein by reacting the corresponding alcohols with malic acid. It is to be understood, however, that such groups may be introduced by all other procedures known in the art and that the invention is not to be limited in any sense by the method of preparation of the said esters.

The following example is presented in order to clearly demonstrate a malic ester of the type contemplated herein.

## Example

Malic acid (20.1 grams; 0.15 mole), oenol (40.2 grams; 0.15 mole) predominantly oleyl alcohol and having a hydroxyl number of 210, and 2-ethyl hexanol (23.5 grams; 0.18 mole) were digested for 3½ hours at 115-120° C. in a flask provided with a reflux take-off. Inasmuch as

some 2-ethyl hexanol distilled out of the reaction mixture into the reflux take-off during digestion, a 0.03 mole excess of 2-ethyl hexanol was used in order to maintain a reaction mixture having substantially equal amounts of the said alcohols. Thereafter, toluene was added to the reaction mixture and the resultant mixture was then refluxed at 140-145° C. for about 7 hours. During the latter period about 4.9 cc. of water was collected in the reflux take-off, evidencing the formation of the ester of malic acid. The reaction mixture was filtered. Toluene was removed from the filtrate obtained thereby, by heating under vacuum to a maximum liquid temperature of 100° C. at 3 mm. pressure. The ester product of malic acid thus obtained had a neutralization number (n. n.) of 20 and is believed to be predominantly one isomeric form or a mixture of both isomeric forms of 2-ethyl hexyl, oleyl malate. It is probable, however, that small amounts of dioleyl malate and di(2-ethyl hexyl) malate are present in the product.

The number of carbon atoms in the aforesaid aliphatic groups and the proportions of the said groups in the malic acid esters of this invention are critical and, if not maintained, esters appreciably inferior to those desired and contemplated are obtained. Esters of malic acid obtained by departing from the aforesaid critical limitations have been found to either fail as rust inhibitors, such as dioleyl malate mentioned above, or cause substantial and deleterious emulsions to form in an environment containing oil and water. This relationship is demonstrated hereinafter by rust and emulsion test results.

To demonstrate the outstanding character of the oil compositions contemplated herein, typical rust and emulsion tests were carried out with a mineral oil, with blends of the mineral oil and small amounts of malic esters of the type defined hereinabove, and with blends of the mineral oil and small amounts of related, inferior malic esters, not contemplated herein. The malic esters so tested are identified by their acidity as measured by their neutralization numbers and by their composition in terms of molar equivalents of short-chain aliphatic groups and of long-chain aliphatic groups. The esters described in the table below as malate mixtures are prepared in the manner shown in the example above wherein definite molar quantities of a long-chain alcohol and of a short-chain alcohol are used to esterify malic acid; and the esters described in the table as physical mixtures are obtained by blending

definite proportions of a long-chain ester of malic acid with definite proportions of a short-chain ester of the same acid. The oil used is a blend of solvent-refined, Mid-Continent residual stock with a solvent-refined, Mid-Continent Rodessa distillate stock and has an A. P. I. gravity of 30.8, a flash point of 445° F. and an S. U. V. of 407.7 seconds at 100° F., and had in admixture therewith, 0.2% of 2,6-ditertiary butyl-4-methyl phenol, a well known antioxidant. The oil is suitable for use in turbines and the like, and the tests run on the oil and oil blends simulate conditions existing in turbine operation and analogous operations.

15 The rust test used involves soaking a small disc of polished steel having a slightly concave surface in the oil under test at 90° F. for 30 minutes, and thereafter placing a drop of distilled water below the surface of the oil and upon the surface of the steel disc. The test is then continued for 24 hours at 90° F. At the end of the latter period the steel disc should not have rust formed thereon in order that the oil pass the test; if rust has formed on the disc during this period, the oil under observation fails the test.

20 The emulsion test used herein is the emulsion test for lubricating oils (Method 320.13) described in the Federal Stock Catalog, section IV, part 5, Federal Specifications VV-L-791b, February, 1942.

25 In this test, 40 cc. of oil under observation and 40 cc. of emulsant, either distilled water or a 1% salt (NaCl) solution, are stirred with a paddle at 1500 R. P. M. for 5 minutes in a 100 cc. cylinder

30 at the prescribed temperature of 130° F. Separation of the emulsion formed therein is observed while the cylinder is kept at the prescribed temperature for a specified time interval. Figures given in the chart provided in the catalog identified above are the actual minutes at which there is no continuous layer of the emulsion remaining between the oil and water. With an oil having a viscosity similar to that of the oil used in this test, specifications require that no continuous layer of emulsion remain at the interface after a 30 minute period.

35 Results of the aforesaid rust and emulsion tests are set forth in the table below. For convenience an asterisk (\*) has been used throughout the table to indicate those oil blends which have failed to pass one or both of the said tests and has also been used to designate those oil blends not contemplated by the present invention.

Table

| A. Chemical Mixtures of 2-ethyl hexyl, oleyl malate |                        | N. N. of Ester | Conc., percent | Rust Test | Emulsion Test   |                  |
|-----------------------------------------------------|------------------------|----------------|----------------|-----------|-----------------|------------------|
| Moles of 2-ethyl hexyl alcohol                      | Moles of oleyl alcohol |                |                |           | Distilled Water | 1% NaCl Solution |
| *2.0                                                | *0                     | 25.0           | 0.2            | Fail*     | 2               | 1                |
| 1.6                                                 | 0.4                    | 22.0           | 0.3            | do*       | 14              | 10               |
| 1.4                                                 | 0.6                    | 22.0           | 0.2            | Pass      | 23              | 11               |
| 1.2                                                 | 0.8                    | 21.0           | 0.2            | do        | 28              | 15               |
| 1.0                                                 | 1.0                    | 20.0           | 0.2            | do        | 29              | 17               |
| 0.9                                                 | 1.1                    | 18.0           | 0.2            | do        | 22              | 13               |
| 0.8                                                 | 1.2                    | 20.0           | 0.2            | do        | 16              | 27               |
| 0.7                                                 | 1.3                    | 17.0           | 0.2            | do        | 20              | 23               |
| *0.6                                                | *1.4                   | 19.0           | 0.2            | do        | 22              | 27               |
| *0.5                                                | *1.5                   | 18.0           | 0.2            | do        | *33             | 30               |
| *0.4                                                | *1.6                   | 18.0           | 0.2            | do        | *32             | 29               |
| *0                                                  | *2.0                   | 14.0           | 0.2            | do        | *39             | 28               |
|                                                     |                        |                |                | do        | *42             | *49              |

| B. Physical Mixtures of—              |                               | N. N. of Ester | Conc., percent | Rust Test | Emulsion Test   |                  |
|---------------------------------------|-------------------------------|----------------|----------------|-----------|-----------------|------------------|
| Di-2-ethyl hexyl malate, mole percent | Dioleyl malate, mole per cent |                |                |           | Distilled Water | 1% NaCl Solution |
| (Minutes for complete separation)     |                               |                |                |           |                 |                  |
| *100                                  | *0                            | 25.0           | 0.2            | Fail*     | 2               | 1                |
| 70                                    | 30                            | 22.4           | 0.2            | do*       | 14              | 10               |
| 40                                    | 60                            | 20.6           | 0.2            | Pass      | 24              | 23               |
|                                       |                               |                |                | do        | 27              | 29               |

| C. Chemical mixtures of 2-ethyl hexyl octadecyl malate |                            | N. N. of ester | Conc., percent | Rust test | Emulsion Test   |                  |
|--------------------------------------------------------|----------------------------|----------------|----------------|-----------|-----------------|------------------|
| Moles of 2-ethyl hexyl alcohol                         | Moles of octadecyl alcohol |                |                |           | Distilled water | 1% NaCl solution |
| (Minutes for complete separation)                      |                            |                |                |           |                 |                  |
| *2.0                                                   | *0                         | 25.0           | 0.2            | Fail*     | 2               | 1                |
| *1.8                                                   | *0.2                       | 24.0           | 0.2            | do*       | 14              | 10               |
| 1.6                                                    | 0.4                        | 22.0           | 0.2            | do*       | 21              | 15               |
| 1.4                                                    | 0.6                        | 21.0           | 0.2            | Pass      | 30              | 14               |
| 1.3                                                    | 0.7                        | 22.0           | 0.2            | do        | 28              | 17               |
| 1.0                                                    | 1.0                        | 21.0           | 0.2            | do        | 23              | 27               |
| 0.9                                                    | 1.1                        | 16.0           | 0.2            | do        | 23              | 18               |
| 0.8                                                    | 1.2                        | 23.0           | 0.2            | do        | 30              | 23               |
| 0.6                                                    | 1.4                        | 20.0           | 0.2            | do        | 23              | 24               |
| *0                                                     | *2.0                       | 19.0           | 0.2            | do        | 28              | ****             |

\*\*1/2 cc. of emulsion after 1 hr.\*

\*\*\*1/4 cc. of emulsion after 1 hr.\*

\*\*\*\*1/8 cc. of emulsion after 1 hr.\*

| D. Physical Mixtures of—               |                                    | N. N. of Ester | Conc., percent | Rust Test | Emulsion Test   |                  |
|----------------------------------------|------------------------------------|----------------|----------------|-----------|-----------------|------------------|
| Di-2-ethyl hexyl malate, mole per cent | Di-octadecyl malate, mole per cent |                |                |           | Distilled Water | 1% NaCl Solution |
| (Minutes for complete separation)      |                                    |                |                |           |                 |                  |
| *100                                   | *0                                 | 25.0           | 0.2            | Fail*     | 2               | 1                |
| *90                                    | *10                                | 24.0           | 0.2            | do*       | 14              | 10               |
| 80                                     | 20                                 | 23.2           | 0.2            | do*       | 21              | 14               |
| 70                                     | 30                                 | 22.4           | 0.2            | Pass      | 30              | 19               |
| 60                                     | 40                                 | 21.7           | 0.2            | do        | 22              | 25               |
| 50                                     | 50                                 | 21.2           | 0.2            | do        | 28              | 30               |
| 20                                     | *50                                | 20.3           | 0.2            | do        | 27              | 30               |
| *20                                    | *80                                | 19.8           | 0.2            | do        | *58             | 21               |
| *10                                    | *90                                | 19.4           | 0.2            | do        | *36             | **               |
| *0                                     | *100                               | 19.0           | 0.2            | do        | 28              | ***              |

\*\*1 cc. of emulsion after 1 hr.\*

\*\*\*1/2 cc. of emulsion after 1 hr.\*

| E. Chemical Mixtures of one mole of malic acid and— |                                | N. N. of Ester | Conc., percent | Rust Test | Emulsion Test   |                  |
|-----------------------------------------------------|--------------------------------|----------------|----------------|-----------|-----------------|------------------|
| Moles of Short-Chain Alcohol                        | Moles of Long-Chain Alcohol    |                |                |           | Distilled Water | 1% NaCl Solution |
| (Minutes for complete separation)                   |                                |                |                |           |                 |                  |
| 1.0 n-hexyl                                         | 1.0 oleyl                      | 22.0           | 0.2            | Fail*     | 2               | 1                |
| 1.0 cyclo-hexyl                                     | do                             | 52.0           | 0.2            | Pass      | 17              | 17               |
| 1.0 n-heptyl                                        | do                             | 13.0           | 0.2            | do        | 18              | 30               |
| 1.0 lauryl                                          | do                             | 26.0           | 0.1            | do        | 13              | 14               |
| 1.0 2-ethyl hexyl                                   | 1.0 dodecyl                    | 22.0           | 0.2            | do        | *48             | *45              |
| Do                                                  | 1.0 7-ethyl-2-methyl undecanol | 47.0           | 0.2            | do        | 24              | 11               |
| Do                                                  | 1.0 hexa-decyl                 | 20.0           | 0.2            | do        | 14              | 14               |
|                                                     |                                |                |                |           | 20              | 22               |

The data in section A of the table above for the oil and for the oil blends containing 0.2% of the various chemical mixtures of 2-ethyl hexyl, oleyl malate effectively demonstrates the superiority of the oil compositions contemplated herein. As shown in section A, the oil alone fails to pass the rust test, although the emulsion characteristics thereof are satisfactory. An oil blend containing di(2-ethyl hexyl) malate also fails to pass the rust test, yet has desirable emulsion characteristics. When the ester product blended in the oil is obtained by reacting one molar equivalent of malic acid with from about 0.7 to about 1.6 molar equivalents of 2-ethyl hexyl alcohol and with from about 1.3 to about 0.4 molar equivalent of oleyl alcohol, the oil blends have desirable rust and emulsion characteristics inasmuch as they readily pass both tests. Yet, when the ester product is obtained by reacting one molar equivalent of malic acid with less than about 0.6 molar equivalent of 2-ethyl hexyl alcohol and with more than about 1.4 molar equivalents of oleyl alcohol, oil blends containing the same fail to pass the emulsion test, although they pass the rust test.

Oil blends containing physical mixtures of the malic acids obtained by blending dioleyl malate and di(2-ethyl hexyl) malate are shown in section B of the table. The results provided therein indicate that effective blends are obtained with 40 through 70 mole per cent of di(2-ethyl hexyl) malate and with 70 through 30 mole per cent of dioleyl malate.

The results shown in section C of the table are similar to those shown in section A, in that the results for chemical mixtures of 2-ethyl hexyl, octadecyl malate have the same critical proportions, namely, from about 0.8 to about 1.6 molar equivalents of the short-chain alcohol, such as 2-ethyl hexyl, and from about 1.2 to about 0.4 molar equivalent of the long-chain alcohol, such as octadecyl. Section D of the table carries results of the said tests with oil blends containing small amounts of physical mixtures of di-octadecyl malate and of di(2-ethyl hexyl) malate. These results also indicate the effectiveness of the ester mixtures falling within the aforesaid critical limits.

Oil compositions containing malic acid esters of the type contemplated herein along with an ester mixture not contemplated—lauryl, oleyl malate—are shown in section E of the table. These results demonstrate the critical nature of the mixture of the aliphatic groups; that is, that one such group should contain from six to eight carbon atoms and another should contain at least twelve carbon atoms. For example, lauryl, oleyl malate contains one aliphatic group having twelve carbon atoms and another having eighteen carbon atoms and when blended in the oil does not pass the emulsion test.

The malic acid esters of this invention may be used in oils in amounts of from about 0.1% to about 1.0% although preferred concentrations are of the order of 0.2% and 0.3%. They may also be used in larger concentrations, of the order of 1% and greater, in cutting oils and the like. These esters may also be used alone in oils and may also be used in oils containing one or more additives. For example, they may be used in oils, with oxidation inhibitors, film strength improving agents, oiliness agents, etc. Typical of such additives are the well known phenols, amines, sulfides, organic compounds containing

phosphorus, organic compounds containing halogen, etc.

It is to be understood that although the invention has been illustrated hereinabove by certain preferred esters and oil blends of the same, it is not to be restricted thereto but is to be broadly construed in the light of the scope of the appended claims.

We claim:

10. 1. A mineral oil composition comprising a viscous mineral oil having in admixture therewith a minor proportion, sufficient to impart anti-rusting characteristics to said oil, of an ester product of malic acid selected from the group consisting of: an ester product of malic acid obtained by reacting one molar equivalent of malic acid with from about 0.8 to about 1.6 molar equivalents of a short-chain aliphatic alcohol having from six to eight carbon atoms and with from about 1.2 to about 0.4 molar equivalent of a long-chain aliphatic alcohol having between twelve and about eighteen carbon atoms; and a mixture of esters of malic acid, one of said esters having two short-chain aliphatic groups containing 25 from six to eight carbon atoms substituted for the carboxylic hydrogen atoms of malic acid and said ester being present in the mixture in a molar quantity of from about forty to about eighty per cent, and another of said esters having two long-chain aliphatic groups containing 30 between twelve and about eighteen carbon atoms substituted for the carboxylic hydrogen atoms of malic acid and said ester being present in the mixture in a molar quantity of from about sixty to about twenty per cent.
2. A mineral oil composition comprising a viscous mineral oil having in admixture therewith a minor proportion, from about 0.01 per cent to about 1.0 per cent, of an ester product of malic acid selected from the group consisting of: an ester product of malic acid obtained by reacting one molar equivalent of malic acid with from about 0.8 to about 1.6 molar equivalents of a short-chain aliphatic alcohol having from six to 45 eight carbon atoms and with from about 1.2 to about 0.4 molar equivalent of a long-chain aliphatic alcohol having between twelve and about eighteen carbon atoms; and a mixture of esters of malic acid, one of said esters having two short-chain aliphatic groups containing from six to eight carbon atoms substituted for the carboxylic hydrogen atoms of malic acid and said ester being present in the mixture in a molar quantity of from about forty to about eighty per cent, and another of said esters having two long-chain aliphatic groups containing between twelve and about eighteen carbon atoms substituted for the carboxylic hydrogen atoms of malic acid and said ester being present in the mixture in a molar quantity of from about sixty to about twenty per cent.
3. A mineral oil composition comprising a viscous mineral oil normally permitting rusting of ferrous metal surfaces in the presence of water, having in admixture therewith a minor proportion, sufficient to retard said rusting, of an ester product of malic acid obtained by reacting one molar equivalent of malic acid with from about 0.8 to about 1.6 molar equivalents of a short-chain aliphatic alcohol having from six to eight carbon atoms and with from about 1.2 to about 0.4 molar equivalent of a long-chain aliphatic alcohol having from twelve to eighteen carbon atoms.
4. A mineral oil composition comprising a vis-

cous mineral oil normally permitting rusting of ferrous metal surfaces in the presence of water, having in admixture therewith a minor proportion, sufficient to retard said rusting, of an ester product of malic acid obtained by reacting one molar equivalent of malic acid with one molar equivalent of a short-chain aliphatic alcohol having from six to eight carbon atoms and with one molar equivalent of a long-chain aliphatic alcohol having from twelve to eighteen carbon atoms.

5. A mineral oil composition comprising a viscous mineral oil normally permitting rusting of ferrous metal surfaces in the presence of water, having in admixture therewith a minor proportion, sufficient to retard said rusting, of an ester product of malic acid obtained by reacting one molar equivalent of malic acid with from about 0.8 to about 1.6 molar equivalents of 2-ethyl hexyl alcohol and with from about 1.2 to about 0.4 molar equivalent of oleyl alcohol.

6. A mineral oil composition comprising a viscous mineral oil normally permitting rusting of ferrous metal surfaces in the presence of water, having in admixture therewith a minor proportion, sufficient to retard said rusting, of an ester product of malic acid obtained by reacting one molar equivalent of malic acid with from about 0.8 to about 1.6 molar equivalents of 2-ethyl hexyl alcohol and with from about 1.2 to about 0.4 molar equivalent of octadecyl alcohol.

7. A mineral oil composition comprising a viscous mineral oil normally permitting rusting of ferrous metal surfaces in the presence of water, having in admixture therewith a minor proportion, sufficient to retard said rusting, of an ester product of malic acid obtained by reacting one molar equivalent of malic acid with from about 0.8 to about 1.6 molar equivalent of 2-ethyl hexyl alcohol and with from about 1.2 to about 0.4 molar equivalent of hexadecyl alcohol.

8. A mineral oil composition comprising a viscous mineral oil normally permitting rusting of ferrous metal surfaces in the presence of water, having in admixture therewith a minor proportion, sufficient to retard said rusting, of a mixture of esters of malic acid, one of said esters having two short-chain aliphatic groups containing from six to eight carbon atoms substituted for the carboxylic hydrogen atoms of malic acid and said ester being present in the mixture in a molar quantity of from about forty to about eighty per cent, and another of said esters having two long-chain aliphatic groups containing from twelve to eighteen carbon atoms substituted for the carboxylic hydrogen atoms of malic acid and said ester being present in the mixture in a molar quantity of from about sixty to about twenty per cent.

9. A mineral oil composition comprising a viscous mineral oil normally permitting rusting of ferrous metal surfaces in the presence of water, having in admixture therewith a minor proportion, sufficient to retard said rusting, of a mixture of esters of malic acid, one of said esters having two short-chain aliphatic groups containing from six to eight carbon atoms substituted for the carboxylic hydrogen atoms of malic acid and said ester being present in the mixture in a molar quantity of about fifty per cent, and another of said esters having two long-chain aliphatic groups containing from twelve to eighteen carbon atoms substituted for the carboxylic hydrogen atoms of malic acid and said ester being present in the mixture in a molar quantity of about fifty per cent.

10. A mineral oil composition comprising a viscous mineral oil having in admixture therewith a minor proportion, at least about 0.01 per cent, of an ester product of malic acid selected from the group consisting of: an ester product of malic acid obtained by reacting one molar equivalent of malic acid with from about 0.8 to about 1.6 molar equivalents of a short-chain aliphatic alcohol having from six to eight carbon atoms and with from about 1.2 to about 0.4 molar equivalent of a long-chain aliphatic alcohol having between twelve and about eighteen carbon atoms; and a mixture of esters of malic acid, one of said esters having two short-chain aliphatic groups containing from six to eight carbon atoms substituted for the carboxylic hydrogen atoms of malic acid and said ester being present in the mixture in a molar quantity of from about forty to about eighty per cent, and another of said esters having two long-chain aliphatic groups containing between twelve and about eighteen carbon atoms substituted for the carboxylic hydrogen atoms of malic acid and said ester being present in the mixture in a molar quantity of from about sixty to about twenty per cent.

GEORGE H. S. SNYDER.

RALPH V. WHITE.

JOHN H. BISHOP.

JOHN F. SOCOLOFSKY.

#### REFERENCES CITED

The following references are of record in the file of this patent:

#### UNITED STATES PATENTS

| Number    | Name       | Date          |
|-----------|------------|---------------|
| 1,993,736 | Graves     | Mar. 12, 1935 |
| 2,101,227 | Werntz     | Dec. 7, 1937  |
| 2,370,299 | Farrington | Feb. 27, 1945 |
| 2,370,300 | Farrington | Feb. 27, 1945 |
| 2,375,516 | Blair, Jr. | May 8, 1945   |

**Certificate of Correction**

February 17, 1948.

Patent No. 2,436,272.

**GEORGE H. S. SNYDER ET AL.**

It is hereby certified that error appears in the printed specification of the above numbered patent requiring correction as follows: Column 7, line 64, for "0.1%" read 0.01%; and that the said Letters Patent should be read with this correction therein that the same may conform to the record of the case in the Patent Office.

Signed and sealed this 4th day of May, A. D. 1948.

[~~seal~~]

**THOMAS F. MURPHY,**  
*Assistant Commissioner of Patents.*